

# UNITED STATES PATENT OFFICE.

PAUL RALPH HERSHMAN, OF CHICAGO, ILLINOIS, ASSIGNOR TO ARMOUR FERTILIZER WORKS, OF CHICAGO, ILLINOIS, A CORPORATION OF NEW JERSEY.

## CONTINUOUS PROCESS OF PRODUCING NITROGENOUS COMPOUNDS OF ALUMINUM.

1,188,770.

Specification of Letters Patent. Patented June 27, 1916.

No Drawing.

Application filed November 25, 1913. Serial No. 803,008.

To all whom it may concern:

Be it known that I, PAUL RALPH HERSHMAN, a citizen of Austria-Hungary, residing at Chicago, in the county of Cook and State 5 of Illinois, have invented certain new and useful Improvements in Continuous Processes of Producing Nitrogenous Compounds of Aluminum, of which the following is a specification.

10 It is a well-known fact that aluminum oxid when mixed with carbon and heated at high temperatures in a current of air or nitrogen, combines with the nitrogen only slowly and incompletely.

15 The leading purpose of the present invention is the provision of a process in the carrying out of which the nitrogen will be taken up quite rapidly and the amount combined largely increased.

20 The preferred manner of carrying out this process is substantially as follows: A mixture of approximately six parts by weight of aluminum oxid, substantially one part by weight of calcium oxid, and approximately 25 four parts by weight of carbonaceous matter, which by decomposition forms minutely divided carbon, is heated in the presence of nitrogen to substantially 1700° to 1800° centigrade, preferably in an 30 electric resistance furnace. The addition of the calcium oxid serves to destroy or eliminate the carbon monoxid formed in the process, the presence of which is quite detrimental to the formation of the desired nitrogenous 35 compounds.

Stated differently, the presence of the carbon monoxid tends to reconvert at lower temperatures the nitrogenous compounds of aluminum into aluminum oxid or carbid, and 40 it is to prevent such reaction that the calcium oxid is used. I have also found that it is of advantage to add a small amount, say one-tenth to one per cent. of a catalytic agent, preferably one capable of combining 45 with nitrogen, such as boron, or titanium, or any of their compounds susceptible to reduction by carbon. Calcium carbid is formed at the beginning of the process, but at the higher temperatures reached it is reconverted 50 into calcium oxid by the carbon monoxid evolved, as expressed in this formula:



Taking  $CH_4$  as a type of carbonaceous

matter and  $AlN$  as a type of nitrogenous 55 aluminum compound, the main reaction is expressed as follows:



The resulting mass contains from 25% to 60 35% of nitrogen, of which part is easily convertible into ammonia by distillation with steam at 100° centigrade, the remainder by distillation with steam at 130° centigrade. The hydroxids of metals left as a residue 65 after the distillation can be dried and calcined. The oxids formed are then ready for another treatment with nitrogen.

I claim:

1. The process of forming nitrogenous 70 compounds of aluminum, consisting in heating in the presence of nitrogen, a mixture of aluminum oxid, a reducing agent, and an ingredient capable of reacting with the carbon monoxid formed, substantially as described.

2. The method of forming nitrogenous 80 compounds of aluminum, which consists in heating in the presence of nitrogen, at a temperature of approximately 1700° to 1800° 80 centigrade, a mixture of aluminum oxid, carbonaceous material, and an ingredient capable of reacting with the carbon monoxid formed, substantially as described.

3. The method of forming nitrogenous 85 compounds of aluminum, which consists in heating in the presence of nitrogen, a mixture of aluminum oxid, carbonaceous material, a catalytic agent capable of combining with nitrogen, and an ingredient capable of 90 reacting with the carbon monoxid formed, substantially as described.

4. The method of producing nitrogenous 95 compounds of aluminum, which consists in heating at a temperature of substantially 1700° to 1800° centigrade, in the presence of nitrogen, a mixture of substantially six parts of aluminum oxid, four parts of carbonaceous matter, one part of calcium oxid, and a small amount of a catalytic agent, substantially as described.

DR. PAUL RALPH HERSHMAN.

Witnesses:

GEO. T. DALE,  
WALDEMAR SILL.